

## 1

2,868,640

## TITANIUM ALLOYS

James Morris Butler, Moseley, Birmingham, England, assignor to The British Non-Ferrous Metals Research Association, London, England, an association of Great Britain

No Drawing. Application January 11, 1955  
Serial No. 481,263

7 Claims. (Cl. 75—175.5)

This invention relates to new and improved titanium base alloys and their use in industry.

For many purposes it is desirable to produce a titanium base alloy capable of being easily hot-worked and possessing good creep-resistant properties at temperatures of the order of 400° C.

## 2

According to the present invention, therefore, a series of valuable titanium base alloys is provided having the following range of composition, namely:

|    |            | Percent, inclusive |
|----|------------|--------------------|
| 5  | Aluminium  | 3 to 10            |
|    | Zirconium  | 1 to 20            |
|    | Silicon    | 0 to 0.5           |
|    | Manganese  | 0 to 5.0           |
|    | Molybdenum | 0 to 5.0           |
| 10 | Vanadium   | 0 to 5.0           |
|    | Titanium   | Remainder          |

In Table I the behaviour of some ternary and quaternary alloys of the invention on hot-working by rolling at 1000° C. and in creep tests at 400° C. and 500° C. is compared with that of some known titanium-aluminium alloys containing silicon or molybdenum but no zirconium. The creep resistance is expressed as the stress in tons/in.<sup>2</sup> required to produce an extension of 1% in 500 hours at the temperature specified.

Table I

| Al, Percent             | Si, Percent | Zr, Percent | Mo, Percent | Mn, Percent | Behaviour on rolling at 1,000° C. |         | Creep test at— |         |
|-------------------------|-------------|-------------|-------------|-------------|-----------------------------------|---------|----------------|---------|
|                         |             |             |             |             | 400° C.                           | 500° C. | 400° C.        | 500° C. |
| Known Alloys            |             |             |             |             |                                   |         |                |         |
| 5.0                     | 0.5         | —           | —           | —           | fair; some edge cracking.         |         | 34-36          | 12-14   |
| 5.0                     | 1.0         | —           | —           | —           | do                                |         | 35-40          | —       |
| 5.0                     | —           | —           | 1           | —           | good                              |         | 25-30          | —       |
| 5.0                     | —           | —           | 5           | —           | do                                |         | 35-38          | 18-20   |
| 5.0                     | —           | —           | 10          | —           | do                                |         | 35-40          | —       |
| Alloys of the Invention |             |             |             |             |                                   |         |                |         |
| 5.0                     | —           | 1           | —           | —           | very good                         |         | 35-40          | —       |
| 5.0                     | —           | 5           | —           | —           | do                                |         | 36-39          | 12-14   |
| 5.0                     | —           | 10          | —           | —           | do                                |         | 40-44          | 14-16   |
| 5.0                     | 0.1         | 5           | —           | —           | good                              |         | 38-41          | 17-19   |
| 5.0                     | 0.25        | 5           | —           | —           | do                                |         | 42-45          | 18-21   |
| 5.0                     | 0.1         | 10          | —           | —           | do                                |         | 38-41          | 18-20   |
| 5.0                     | —           | 10          | 1           | —           | do                                |         | 45-47          | 15-17   |
| 5.0                     | —           | 5           | 1           | —           | moderate                          |         | 43-45          | 15-17   |

In a paper entitled "Titanium Alloy Development" presented by M. Hansen and H. D. Kesseler in January 1953, to the American Society of Automotive Engineers, the properties of titanium base alloys in current use are described and these authors show that certain titanium-aluminium-molybdenum and titanium-aluminium-silicon alloys are among the most creep-resistant titanium base alloys known to date.

We have now found that titanium base alloys consisting (apart from iron, nitrogen, oxygen and carbon which may be adventitiously present and must not exceed 0.25% each) of from 3-10% of aluminium and from 1-20% zirconium, the balance being titanium, exhibit a markedly better combination of hot-working properties and creep-resistance than titanium base alloys in use heretofore.

We have also found that these properties are still further enhanced by the inclusion of one or more of the following components, namely:

|            | Percent   |
|------------|-----------|
| Silicon    | Up to 0.5 |
| Manganese  | Up to 5.0 |
| Molybdenum | Up to 5.0 |
| Vanadium   | Up to 5.0 |

the balance in each case being titanium.

The superiority of the alloys of the invention is evident. The ternary titanium-aluminium-zirconium alloys show a markedly better combination of hot-working properties and creep-resistance than the known titanium base alloys and the quaternary alloys combine a good behaviour on hot-rolling with a very good creep-resistance especially at 500° C.

Moreover these quaternary alloys have a superior ductility in the as-rolled condition as compared with known titanium-aluminium-molybdenum or titanium-aluminium-silicon alloys, the ductility of which is not readily improved by heat-treatment.

In the quaternary alloys part of the silicon, manganese, molybdenum, or vanadium may be replaced by one or more of the other three components and, provided the total composition is within the range above specified, the multi-component alloys have similarly enhanced properties.

Table II shows the results of creep tests on three titanium base alloys containing 5.0% aluminium and, respectively, 5% of molybdenum, 0.5% of silicon and 10% of zirconium, the results being expressed as percentage strains after 300 hours at 400° C. under stresses of 25 and 20 tons per square inch.

3  
Table II

| Titanium alloys containing |             |             |             | Percent Strain after 300 Hrs. at 400° C. under stress of— |                          |
|----------------------------|-------------|-------------|-------------|-----------------------------------------------------------|--------------------------|
| Al, Percent                | Si, Percent | Mo, Percent | Zr, Percent | 25 tons/in. <sup>2</sup>                                  | 20 tons/in. <sup>2</sup> |
| 5.0                        | —           | 5.0         | —           | 0.16                                                      | 0.12                     |
| 5.0                        | 0.5         | —           | —           | 0.12                                                      | 0.05                     |
| 5.0                        | —           | —           | 10.0        | 0.06                                                      | 0.03                     |

The superiority of the titanium-aluminium-zirconium alloy of the invention is apparent.

The low density and relatively high resistance to creep of the alloys of the invention make them attractive for use in industry, e. g. for gas turbine and other engine components which are required to operate at temperatures up to about 400° C., particularly where such components are subjected in service to stresses arising from inertia forces.

I claim:

1. An engine component capable of withstanding about 400° C. which is required to have high creep resistance due to inertia forces and which is made of a titanium base alloy which, apart from iron, nitrogen, oxygen and carbon present in amounts not exceeding 0.25% each, consists essentially of about: 3 to 10% aluminum, 1 to 20% zirconium with at least one metal of the group consisting of silicon, manganese, molybdenum and vanadium present in amounts up to 0.5% in the case of silicon, up to 5% in the case of manganese, up to 5% in the case of molybdenum and up to 5% in the case of vanadium, the creep resistance of the alloy being at least 40 tons per square inch at 400° C.

2. A titanium base alloy which apart from iron, nitrogen, oxygen and carbon present in amounts not exceeding 0.25% each, consists essentially of about 3 to 10% aluminum, 1 to 20% zirconium with at least one metal of the group consisting of silicon, manganese, molybdenum and vanadium present in significant amounts up

to 0.5% in the case of silicon, up to 5% in the case of manganese, up to 5% in the case of molybdenum and up to 5% in the case of vanadium, the creep resistance of the alloy being at least 40 tons per square inch at 400° C.

5 3. A titanium base alloy consisting of, apart from iron, nitrogen, oxygen and carbon present in amounts not exceeding 0.25% each, 5% of aluminum and 5% of zirconium, together with 0.1% of silicon, the remainder being titanium.

10 4. A titanium base alloy consisting of, apart from iron, nitrogen, oxygen and carbon present in amounts not exceeding 0.25% each, 5% of aluminum and 5% of zirconium, together with 0.25% of silicon, the remainder being titanium.

15 5. A titanium base alloy consisting of, apart from iron, nitrogen, oxygen and carbon present in amounts not exceeding 0.25% each, 5% of aluminum and 10% of zirconium, together with 0.1% of silicon, the remainder being titanium.

20 6. A titanium base alloy consisting of, apart from iron, nitrogen, oxygen and carbon present in amounts not exceeding 0.25% each, 5% of aluminum and 10% of zirconium, together with 1% of manganese, the remainder being titanium.

25 7. A titanium base alloy consisting of, apart from iron, nitrogen, oxygen and carbon present in amounts not exceeding 0.25% each, 5% of aluminum, 5% of zirconium, together with 1% of molybdenum, the remainder being titanium.

#### References Cited in the file of this patent

##### UNITED STATES PATENTS

|           |               |       |               |
|-----------|---------------|-------|---------------|
| 2,669,513 | Jaffee        | ----- | Feb. 16, 1954 |
| 2,703,278 | Finlay et al. | ----- | Mar. 1, 1955  |
| 2,704,251 | Vordahl       | ----- | Mar. 15, 1955 |
| 2,754,204 | Jaffee et al. | ----- | July 10, 1956 |
| 2,754,205 | Jaffee et al. | ----- | July 10, 1956 |

##### FOREIGN PATENTS

|         |         |       |               |
|---------|---------|-------|---------------|
| 718,822 | Germany | ----- | Feb. 26, 1942 |
|---------|---------|-------|---------------|